

1

3,817,751

**COLOR FORMING AGENTS FOR THE PEROXIDE COLOR INTENSIFYING PROCESS**  
Reinhart Matejec and Walter Puschel, Leverkusen, Germany, assignors to Agfa-Gevaert Aktiengesellschaft, Leverkusen, Germany  
No Drawing. Filed Apr. 21, 1972, Ser. No. 246,387  
Claims priority, application Germany, Apr. 24, 1971,

P 21 20 091.9  
Int. Cl. G03c 1/00

U.S. Cl. 96—48 R

2 Claims

### ABSTRACT OF THE DISCLOSURE

Process for the production of photographic dye images by imagewise decomposition of peroxide compounds in the presence of reactants for a color forming oxidation coupling reaction wherein the reactants are organic compounds which contain a CN single or double bond and in which the carbon atom is substituted with a hydroxy- or amino-substituted aryl group and the nitrogen atom is substituted with a hydroxy- or amino-substituted aryl group or is a ring member of a heterocyclic saturated or unsaturated 5- or 6-membered ring.

The invention relates to a process for the production of photographic images by imagewise decomposition of peroxide compounds in the presence of compounds for a color forming oxidation reaction.

The production of photographic images by imagewise production of compounds which catalyse the decomposition of peroxide compounds followed by imagewise formation of dyes by oxidative coupling is known per se. By catalytic decomposition is meant here the catalytic activation of the peroxide which is required for the color forming oxidation reaction.

In this process a light-sensitive layer is exposed imagewise to produce in imagewise distribution nuclei of noble metals of Groups Ib and/or VIII of The Periodic Table. The layer containing the nuclei is then treated with peroxide compounds which decompose catalytically at the nuclei in the image areas in the presence of reactants for a color forming oxidation reaction.

Instead of using light-sensitive layers which on exposure form metal nuclei which will decompose peroxide compounds, the layers used for the above mentioned process for the production of photographic images may contain substances which yield other peroxidase active catalyst on exposure. Suitable for this process are, for example, certain complex compounds of heavy metals of Groups VIIb, VIIb and VIII of The Periodic Table with a mono-basic or polybasic carboxylic acid or other ligands. Compounds which split off iodine ions on exposure to light have the same effect.

The process may also be carried out with light-sensitive photographic materials which contain, uniformly distributed, catalase active enzymes such as catalase, peroxidase, haemoglobin or haemin which are inactivated in the image areas when exposed to actinic light. Direct positive images are obtained with these materials.

It is among the objects of the present invention to improve the above described process for the production of photographic dye images by means of new reactants for the oxidative coupling reaction, in order to increase in velocity of dye formation, the color density and the stability of the dye image.

We now have found a process for the production of photographic images including the steps of imagewise ex-

2

posing a light-sensitive layer to form nuclei which decompose peroxide compounds followed by treatment with catalytically decomposable peroxide compounds in the presence of reactants for a color forming oxidative coupling reaction wherein the color forming reactants are organic compounds which contain a CN single or double bond and in which the carbon atom is substituted with a hydroxy-substituted or amino-substituted aryl group and the nitrogen atom is substituted with a hydroxy-substituted or amino-substituted aryl group or is a ring member of a heterocyclic saturated or unsaturated 5- or 6-membered ring.

Reactants of the following general formulae have proved to be especially suitable:



wherein

20  $R_1$ =aryl substituted with hydroxyl and/or amino groups, especially phenyl, which aryl groups may also contain additional substituents, e.g. alkoxy having up to 18 preferably up to 5 carbon atoms, halogen such as chlorine, bromine or iodine, alkyl groups having up to 18 and preferably up to 3 carbon atoms, sulfo, esterified sulfo, carboxyl or esterified carboxyl or nitrile;

25  $R_2$ =hydrogen, alkyl having up to 18, preferably up to 5 carbon atoms which may contain additional substituents, e.g. carboxyl or hydroxyl or aryl, in particular phenyl in which the phenyl ring may contain the substituents listed under  $R_1$ ;

30  $R_3$  and  $R_4$  have the same meaning as  $R_2$ ;

$R_5$  has the same meaning as  $R_1$ ;

35 or alternatively

35  $R_1$  and  $R_5$  and/or  $R_4$  and  $R_5$  may also denote the ring members required to complete a heterocyclic saturated or unsaturated 5-membered or 6-membered ring which contains nitrogen.

The nitrogen atom of the CN-bond in the above formulae may be present in quaternized form.

Particular utility is exhibited by the following compounds:





3,817,751

24

5



25



26



27



28



29



30



31



32



33



34

6



35



36



37



38



39



40



41



42



43



75



The above compounds are prepared by known processes. The preparation of some of these compounds is described in detail below; the others are obtained by analogous methods.

Compound 1

7.3 g. of vanillin and  
 5.6 g. of 4,4'-diamino-diphenylaminosulfonic acid-(2) in  
 50 ml. of pyridine with the addition of  
 5 ml. of triethylamine are heated on a steam bath for one  
 hour. Pyridine is distilled off under vacuum and the  
 residue is redissolved in  
 25 ml. of pyridine whilst hot. After cooling,  
 100 ml. of isopropanol are added and the reaction mix-  
 ture is filtered over active charcoal.  
 50 ml. of glacial acetic acid and  
 100 ml. of isopropanol are added to the filtrate. After one  
 hour, the filtrate is suction-filtered and immediately  
 stirred up with water.

Compound 4

10 g. of vanillin and  
 8.1 g. of 4,4'-diaminodiphenylamine in  
 100 ml. of pyridine are heated on a steam bath for 30  
 minutes with stirring. The reaction mixture is filtered  
 whilst hot and the pyridine is distilled off under vac-  
 um. The residue is triturated with ethyl acetate and  
 again suction filtered.

Yield: 12.5 g.; M.P.: 194-196° C.

The preparation of compounds 6-43 has been described in British Patent Specification No. 1,210,417.

The compounds disclosed in U.S. Patent Specification No. 3,535,114 are also suitable; compound 45 is an example thereof.

Some of the above compounds are already known as photographic developing agents. Of course one can only use compounds as photographic developing agents which have a suitable redox potential in the required pH region, i.e. which are capable of reducing silver halides to metallic silver.

The use of these substances for the purpose of the invention is completely different from their known use as photographic developers. According to the invention, these substances are used as reactants for a color forming coupling reaction which requires the decomposition of the peroxide compound as oxidizing agent. The oxidative coupling reaction has nothing whatever to do with the photographic development of exposed silver halide. Consequently, when these substances are used in accordance with this invention, they are not required to satisfy any conditions as regards their activity within certain, relatively narrow pH ranges.

However for catalytic dye formation the color forming agents must also satisfy certain requirements as regards their electrochemical properties. Thus, they should have an anodic redox potential which is more negative at the pH values employed than the cathodic redox potential of the peroxide compound used, with the additional requirement that the difference between these two redox potentials must not exceed the value which corresponds to the

activation energy required for the (non-catalytic) decom-  
 position of the peroxy compound. However, these activation  
 energies (and hence also the permissible potential  
 differences) are very high and furthermore it is possible  
 by suitable choice of various inorganic and/or organic  
 peroxy compounds to cover an almost unlimited range of  
 potentials. Hence even those compounds of structural for-  
 mulae (I) and (II) which are not operative as photo-  
 graphic developers are suitable for use as color forming  
 agents for the catalytic dye formation.

These substances which cannot be used as photographic  
 developers yield, for example, brownish black to black  
 dyes by catalytic dye formation on the image silver by  
 decomposition of the peroxy compound, in particular  
 H<sub>2</sub>O<sub>2</sub>.

The substances for use according to the invention may  
 also be used in admixture with other reactants, e.g. pyro-  
 catechol, resorcinol, ortho- and para-phenylene diamines,  
 diamine, N-allyl- and N,N-dialkyl-phenylenediamine.  
 20 Further improvement in dye formation can thereby be ob-  
 tained. These substances have been described e.g. in  
 British Patent Specification No. 1,268,126 or U.S. Ser. No.  
 881,610 now U.S. Pat. No. 3,674,490.

Production of the photographic images may be carried  
 25 out in various ways by known methods. It is practically  
 immaterial which peroxides active catalysts distributed in  
 accordance with the image are used for the imagewise  
 activation of the peroxide compound. It is preferred to use  
 layers which upon exposure produce imagewise nuclei of  
 30 noble metals of the Groups IB and/or VIII of The  
 Periodic Table which in turn catalytically accelerate the  
 decomposition of the peroxide compound. Photographic  
 materials of this kind have been described in the above  
 British Patent Specification.

35 Another suitable method of decomposing peroxide com-  
 pounds imagewise has been described in British Patent  
 Application No. 46,694/70 and U.S. Patent Application  
 Ser. No. 74,482. The said Patent Applications relate to a  
 40 light-sensitive material which contains compounds which  
 on exposure to light form catalase active and/or peroxy-  
 dase active catalysts. These are complex compounds of  
 metals of Groups VIB, VIIIB or VIII of The Periodic  
 Table of Elements.

A similar material has been described in British Patent  
 45 Application 57,633/70 and U.S. Patent Application Ser.  
 No. 94,573 now U.S. Pat. No. 3,684,511. According to  
 the said Patent Applications, the light-sensitive layer  
 contains a compound which splits off catalase active or  
 peroxydase active iodine ions on exposure to light.

50 Another possible method has been described in British  
 Patent Application No. 51,141/70 and U.S. Patent Ap-  
 plication Ser. No. 84,195 now U.S. Pat. No. 3,694,207.  
 The material described there enables direct positive images  
 to be produced. The light-sensitive layer contains catalase  
 55 active and/or peroxydase active enzymes which are in-  
 activated on exposure to light. The material is then treated  
 with hydrogen peroxide, decomposition then taking place  
 only in the areas which have not been struck by light.

Suitable peroxide compounds are e.g. inorganic peroxide  
 60 compounds such as perborates, percarbonates, persilicates,  
 perphosphates or persulfates. Organic peroxide com-  
 pounds may also be used, e.g. benzoyl peroxide. Hydrogen  
 peroxide is particularly suitable owing to its efficient action  
 65 and the ease with which it can be handled in the form of  
 aqueous solutions. Especially useful are addition com-  
 pounds of hydrogen peroxide with organic compounds,  
 especially urea, acid amides, polyhydroxyl compounds or  
 amines.

EXAMPLE 1

70 5 litres of an 8% aqueous gelatin solution are added  
 to 1 litre of a highly sensitive silver iodobromide gelatin  
 emulsion (4.5 mol-percent/AgI). The mixture is adjusted  
 to pH 5.5. 200 g. of compound 44 are then suspended in  
 this mixture which is then cast on a support of poly-

ethylene terephthalate (layer thickness approx.  $5\mu$ , silver application approximately 1.5 g. of Ag/m<sup>2</sup> in the form of silver halide).

This layer is then covered with a protective gelatin layer about  $8\mu$  in thickness. The layer is then hardened by treatment with an aqueous solution of formalin or mucochloric acid in the usual manner.

After imagewise exposure (0.5 seconds with X-rays between fluorescent intensifying foils) the layer is immersed in the following developer solution for 10 seconds at 35° C.:

Bath I:

2 g. of 1-phenylpyrazolidone-3  
25 g. of hydroquinone  
100 g. of anhydrous Na<sub>2</sub>SO<sub>3</sub>  
1 g. of polyethylene oxide wax made up to 1 litre with H<sub>2</sub>O adjusted to pH 11.5 with NaOH.

After brief washing, the layer is immersed for 10 seconds in a mixture of the following composition at 35° C.:

Bath II:

700 cc. of 30% aqueous H<sub>2</sub>O<sub>2</sub>  
300 cc. of isopropanol  
5 cc. of acetone.

In this bath, a black dye image (negative of the exposure original) is produced catalytically on the image silver with the aid of the peroxide introduced into the layer.

The layer is finally stabilized and fixed by introducing it for 10 seconds into a solution of the following composition at 35° C.:

Bath III:

100 g. of Na<sub>2</sub>S<sub>2</sub>O<sub>3</sub>  
2 g. of KSCN  
20 g. of Al<sub>2</sub>(SO<sub>4</sub>)<sub>3</sub>·18H<sub>2</sub>O in 1 litre of H<sub>2</sub>O adjusted pH 12 with NaOH.

This bath III stabilizes the dye image to such an extent that subsequent washing is not absolutely necessary. A brief final washing (e.g. 10 seconds) is recommended only if the images are to be stored for a long time (e.g. longer than 2 months).

The color density of the dye image can be increased by briefly heating the layer between bath II and bath III (e.g. by infra-red radiation for 10 seconds at about 80° C.).

EXAMPLE 2

Preparation of the light-sensitive material:

20 g. of green ammonium ferric citrate are dissolved in 80 cc. of water  
6 g. of ammonium ferrioxalate are dissolved in 60 cc. of water  
5 g. of K<sub>3</sub>Fe(CN)<sub>6</sub> are dissolved in 50 cc. of water  
1 g. of citric acid is dissolved in 10 cc. of water  
12 g. of gelatin are dissolved in 200 cc. of water.

The above solutions are mixed together in red darkroom light and the mixture is cast on a support of cellulose triacetate. The thickness of the dried layer is about 10 to 20 $\mu$ . The layer is hardened in the usual manner, by addition of a 2 ml. of a 30% aqueous solution of formalin or mucochloric acid.

Processing: The dried layer is exposed imagewise behind a grey step in a conventional sensitometer (100 watt lamp, exposure time 10 seconds). It is then exposed to a water vapour atmosphere at about 80° C. for about 10 to 20 seconds and then hardened for 30 seconds by spraying water on it.

The layer is then introduced into a bath (I) of the following composition for 30 seconds:

Bath I:

5 500 cc. of 30% H<sub>2</sub>O<sub>2</sub>  
500 cc. of a saturated aqueous solution of 1-phenyl-ethanol  
25 g. of the sodium salt of benzilic acid.

It is then treated for 30 seconds with

10 Bath II:

16 g. (N,N-diethyl)p-phenylenediaminsulfate  
20 g. of compound 1  
9 g. of sodium sulfite made up to 1 litre with H<sub>2</sub>O adjusted to pH 9.5 with K<sub>2</sub>CO<sub>3</sub>.

It is then stabilized by immersing it for 30 seconds into a solution of

Bath III:

20 25 g. of ZnSO<sub>4</sub>·7H<sub>2</sub>O in 1 litre of H<sub>2</sub>O with citric acid/citrate buffer adjusted to pH 5.

A black negative image of the original is obtained.

EXAMPLE 3

25 A transparent support of cellulose triacetate is coated with a solution containing 6 ml. of a 10% aqueous solution of polyvinyl alcohol and 2 g. of TiO<sub>2</sub> reduced to a particle size of 0.3 to 0.4  $\mu$ m. and 0.1 mg. of erythrosine as spectral sensitizer in 400 cc. of water. The layer is then dried.

30 The dried layer is exposed imagewise and then treated for 30 seconds in the following bath at 20° C.:

Bath I: 2% aqueous NaPd(C<sub>2</sub>O<sub>4</sub>)<sub>2</sub> solution.

35 After brief washing, the layer is introduced for 30 seconds into a solution of the following composition at 20° C.:

Bath II:

40 500 cc. of 30% H<sub>2</sub>O<sub>2</sub>  
450 cc. of cyclohexanol  
40 cc. of cyclohexanone and  
10 cc. of ethyl methyl glycol.

45 The layer is then introduced for 30 seconds into a bath of the following composition at 20° C. to effect catalytic dye formation:

Bath III:

50 10 g. of compound 45  
50 g. of pyrocatechol  
9 g. of anhydrous Na<sub>2</sub>SO<sub>3</sub> made up to 1 litre with H<sub>2</sub>O adjusted to pH 8 with Na<sub>2</sub>CO<sub>3</sub>.

The layer is finally stabilized by introducing it for 30 seconds into the following solution at 20° C.:

55 12 g. of lead acetate in 1 liter of H<sub>2</sub>O

(adjusted to pH 6 with acetate/acetic acid buffer). A deep black image of the original is obtained.

60 We claim:

1. In a process for the production of photographic images by imagewise exposure of a lightsensitive layer wherein noble metal nuclei are producible, producing in the layer in imagewise distribution nuclei of noble metals of Groups Ib and VIII of The Periodic Table of Elements capable of catalytically decomposing peroxy compounds, treating the layer which contains the imagewise distributed noble metal nuclei in the presence of a color forming compound which on oxidation yields a dye, with a peroxy compound thereby catalytically decomposing said peroxy compound on the noble metal nuclei and oxidizing said color forming compound to yield a dye image, wherein the improvement comprises the color forming compound is an organic compound having an anodic redox potential

70 more negative than the cathodic redox potential of the

75

11

peroxy compound and containing a CN single or double bond according to the following formulae:



5

wherein

$R_1$ =aryl substituted with hydroxyl and/or amino groups

$R_2$ =hydrogen, alkyl or aryl

$R_3$  and  $R_4$  have the same meaning as  $R_2$

$R_5$  has the same meaning as  $R_1$

or alternatively

$R_1$  and  $R_5$  and/or  $R_4$  and  $R_5$  may also denote the ring members required to complete a heterocyclic saturated or unsaturated 5-membered or 6-membered ring.

10

15

12

2. The process of claim 1, wherein the color forming component is reacted in admixture with other aromatic amines, phenols and/or aminophenols.

References Cited

UNITED STATES PATENTS

|           |         |                 |       |          |
|-----------|---------|-----------------|-------|----------|
| 3,674,490 | 7/1972  | Metejec         | ----- | 96-48 PD |
| 3,503,744 | 3/1970  | Itano           | ----- | 96-48 R  |
| 3,697,275 | 10/1972 | Hayakawa et al. | ----- | 96-48 R  |

RONALD H. SMITH, Primary Examiner

J. L. GOODROW, Assistant Examiner

U.S. CL. X.R.